

## UNITED STATES PATENT OFFICE

2,123,152

## TREATMENT OF CELLULOSIC MATERIALS

Georges Rivat, Lyons, France, assignor to Henry Dreyfus, London, England

No Drawing. Application November 5, 1935, Serial No. 48,283. In France November 13, 1934

11 Claims. (Cl. 8—5)

The present invention relates to improvements in the coloration of textile materials, especially cellulosic materials.

As is well known, materials consisting of natural or regenerated cellulose have an affinity for the cotton colors and little or no affinity for the acid colors. Basic colors are usually dyed or printed on such materials with the aid of a tannin mordant. In a similar way, cellulose acetate artificial silk has an affinity for the basic colors and little or no affinity for the acid and direct cotton colors. The present invention is concerned with treating materials made of or containing natural or regenerated cellulose or cellulose derivatives for the purpose of modifying the existing dyeing affinities of these materials and with fixing dyestuffs on the materials. Cellulosic materials may be, for example, natural cellulose fibers such as cotton, linen, jute or ramie, or regenerated cellulose as, for example, viscose, cuprammonium and nitrocellulose artificial silks, or cellulose derivatives, for example cellulose acetate, cellulose formate, cellulose propionate or other esters of cellulose, or cellulose ethers, for example methyl, ethyl or benzyl cellulose, or mixed cellulose derivatives, for example mixed ethers, mixed esters or mixed ether-esters. Again animal fibers, e. g. natural silk, may be colored by the new process.

Broadly the invention comprises incorporating in the materials a complex nitrogen-containing organic compound, preferably of resin character, by interaction, on the materials, of two or more appropriate reagents, one or more of which contain the requisite nitrogen. A dyestuff is applied to the materials either in admixture with one or more of the reagents or separately at a later stage, e. g. after the formation of the complex nitrogenous organic compound on the material.

Incorporation of the complex nitrogen-containing organic compounds in natural or regenerated cellulose by the above method generally confers upon the latter an affinity, or increases any existing affinity, for the basic and acid colors, and decreases or suppresses entirely their affinity for the direct cotton colors. Viewed from the point of view of the basic and acid colors, the invention may therefore be considered as a mordanting of the materials, while from the point of view of the direct cotton colors, it may be considered as a reserving process. Similar observations apply, mutatis mutandis, to the cellulose derivative materials.

The reagents capable of yielding the complex nitrogenous compound may be applied uniform-

ly over the entire material as, for example, by applying them by a bath treatment or by mechanical impregnation methods, for example by means of a padding mangle, but the most important application of the new process consists in modifying the dyeing affinities of the materials under treatment locally so as to produce pattern effects. By such local application, fabrics or other materials may be produced having the property of producing cross-dyed effects directly. For example immersion of such materials in a single bath containing, for example, either an acid or a direct cotton dye produces a fabric having a coloration only locally on the material, either the treated portion or the untreated portion of the material remaining uncolored according to the character of the dyestuff applied.

Again by applying a dyestuff in admixture with the resin-forming reagents valuable fast colorations, uniform or local, may be produced, for example with dyestuffs having normally no affinity for the material.

If desired the coloring matter may also be applied locally, so as to fall at least in part on parts of the material to which the reagents have been applied. A wide range of pattern effects may thus be produced. For example a fabric printed with the reagents in an "all-over" pattern, e. g. of small spots or the like, may be over-printed in a large floral or geometric pattern with a dyestuff having affinity for either the unprinted material or for the complex nitrogenous compound.

As previously indicated, the invention particularly contemplates the incorporation in the materials of synthetic resins containing nitrogen. The synthetic resins may, for example, be produced by the condensation of aldehydic, or ketonic bodies, for example formaldehyde, acetaldehyde, benzaldehyde, acetone or the like, with aliphatic or aromatic amines or amides, for example urea, thiourea, guanidine and their derivatives, dicyandiamide, aniline, methyl aniline, diphenylamine, benzyl aniline,  $\beta$ -naphthylamine, para-toluene-sulphonamide or other aromatic sulphonamides or N-alkyl or other derivatives thereof. A further group of materials available is the condensation products of gelatine, casein or other albumenoid compounds with formaldehyde for example. The invention is not, however, confined to condensation products of aldehydic or ketonic bodies with nitrogen-containing organic compounds, since any other nitrogen-containing resinous or highly complex organic compound is suitable. For example, the condensation product of phenol with methylene diphenyldiamine

may be employed. In most cases, condensation to produce the above mentioned resinous materials is most advantageously carried out in the presence of catalysts, which may be alkaline, acid or neutral.

It is desirable that the nitrogenous product produced by interaction of the reagents on the material shall be substantially insoluble in water or in aqueous reagents which are customarily applied to the textile materials as, for example, in dyeing or scouring operations.

The reagents necessary may be applied together to the materials or may be applied separately or in any suitable combination. For example the fabric may be first impregnated with a catalyst and the mixture of two bodies for condensation subsequently applied, or alternatively the mixture of the two bodies to undergo condensation may be first applied and the catalyst subsequently applied. One of the bodies to be condensed may be applied with the catalyst and the other body applied separately. This last alternative is specially useful where one of the reagents is to be applied in the form of vapor as may be the case, for example, with formaldehyde.

Reaction between the resin-forming reagents is conveniently effected by heating the materials impregnated with the reagents. Steaming may be utilized if desired.

The following examples illustrate the invention.

*Example 1*

A cellulose or cellulose derivative fiber or fabric is impregnated locally or printed or treated in an analogous manner with a mixture having the following composition, the parts being by weight:

|                       | Grams   |
|-----------------------|---------|
| 10) Thiourea-----     | 100-150 |
| Water-----            | 250-300 |
| 40% formaldehyde----- | 550     |
| Formic acid-----      | 50      |

The material is then dried at 80° during an hour or two until the condensation has given rise to a product insoluble in boiling water.

The material thus treated can then be dyed by any suitable process with a direct dyestuff which reserves animal fibers. The dyebath may contain any of the usual assistants, for example a sulphonated higher fatty alcohol or other wetting agent or sodium sulphate. The untreated parts of the material take the color normally while the treated parts act as a reserve against the color so that a white pattern on a colored background is obtained.

In a similar way the material may be dyed with an acid color by choosing an acid dyestuff which has good reserve properties for cotton fibers. The treated parts only are dyed so that a colored pattern on a white background is obtained.

Again, basic dyestuffs may be employed to color the material. In this case, natural or regenerated cellulose materials and also cellulose derivative materials having a certain affinity for these colors, the untreated parts also take some of the color while the treated parts have their affinity for the color enhanced so that deep designs on a paler background are obtained.

A plurality of acid, basic and cotton colors may be applied to the materials in succession or, where they are compatible, in a single bath, so as to obtain differential colorations on the design and background.

*Example 2*

A cellulose or cellulose derivative fiber or fabric is impregnated locally or printed or treated in an analogous manner with the following mixture:

|                             | Grams   |
|-----------------------------|---------|
| Dicyandiamide-----          | 100-200 |
| Ammonium sulphocyanide----- | 20      |
| 40% formaldehyde-----       | 780 10  |

The sequence of operations is carried out as indicated in Example 1.

In the above examples, any other suitable nitrogen-containing bodies may be substituted for the agents therein mentioned. In addition, penetrating agents, plasticizers or softeners such as glycerine, oils, sulphonated fatty oils or the like may be added to the mixture. Latex or other suitable agents having the effect of increasing the fixation of the material may likewise be present. If desired, the mixture for producing the condensation product on the material may contain the dyestuff.

*Example 3*

The cellulose or cellulose derivative fiber or fabric is impregnated locally or printed or treated in an analogous manner with the following mixture:

|                                               | Grams   |
|-----------------------------------------------|---------|
| Urea-----                                     | 100-200 |
| Dicyandiamide-----                            | 60      |
| Glycerine-----                                | 60      |
| Alkaline or alkaline earth sulphocyanide----- | 20 35   |
| 40% formaldehyde-----                         | 660     |

The sequence of operations is effected as indicated in Example 1.

*Example 4*

A fabric of natural silk or regenerated artificial silk is printed with the following mixture:

|                                             |               |         |
|---------------------------------------------|---------------|---------|
| Urea or thiourea-----                       | grams         | 100     |
| 40% formaldehyde-----                       | ccs           | 300-500 |
| Formic acid-----                            | do            | 50      |
| Dyestuff-----                               | grams         | 10-50   |
| Water and thickener sufficient to make 1000 | grams in all. | 50      |

After drying the fabric is stoved at 110° C. for 1-2 hours and then washed with water.

By mixing in the fabric or other material natural silk, wool or other animal fibers, effects due to the weaving or other arrangement of these animal fibers in the goods may be superimposed upon the effects described above.

The following are examples of coloring matters which may be used according to the invention.

| Acid coloring matters | Color index No. |
|-----------------------|-----------------|
| Milling Yellow-----   | 195             |
| Milling Red-----      | 344             |
| Milling Blue-----     | 289 65          |
| Metanil Yellow-----   | 138             |
| Tartrazine -----      | 640             |
| Orange II-----        | 151             |
| Sulpho Green-----     | 669, 670        |
| Acid Fuchine-----     | 692 70          |
| Alkali Blue-----      | 704             |
| Ponceau for silk----- | 196             |
| Acid Violet-----      | 698             |
| Polar Red-----        | 430             |
| Cyanol -----          | 715 75          |

| Basic coloring matters                                                                                                                                                                                                                                                                                                                                                                                               | Color index No. | reacting with formaldehyde to yield a nitrogenous resin, effecting formation of said nitrogenous resin on the material, and thereafter dyeing the material with a dyestuff having affinity for animal fibers.                                                                                                                                                 |
|----------------------------------------------------------------------------------------------------------------------------------------------------------------------------------------------------------------------------------------------------------------------------------------------------------------------------------------------------------------------------------------------------------------------|-----------------|---------------------------------------------------------------------------------------------------------------------------------------------------------------------------------------------------------------------------------------------------------------------------------------------------------------------------------------------------------------|
| Rhoduline Yellow                                                                                                                                                                                                                                                                                                                                                                                                     | 815             |                                                                                                                                                                                                                                                                                                                                                               |
| Acridine Orange                                                                                                                                                                                                                                                                                                                                                                                                      | 788             |                                                                                                                                                                                                                                                                                                                                                               |
| Chrysoidine                                                                                                                                                                                                                                                                                                                                                                                                          | 20              |                                                                                                                                                                                                                                                                                                                                                               |
| 5 Methylene Blue                                                                                                                                                                                                                                                                                                                                                                                                     | 922             |                                                                                                                                                                                                                                                                                                                                                               |
| Toluidine Blue                                                                                                                                                                                                                                                                                                                                                                                                       | 925             | 5. Process of coloring textile fabric containing cellulose filaments, which comprises locally impregnating the material with a mixture containing formaldehyde and urea, heating the fabric to effect resin formation on the material by interaction of the formaldehyde and urea, and dyeing the material with a dyestuff having affinity for animal fibers. |
| Rhoduline Blue                                                                                                                                                                                                                                                                                                                                                                                                       | 658             |                                                                                                                                                                                                                                                                                                                                                               |
| Victoria Blue                                                                                                                                                                                                                                                                                                                                                                                                        | 729             |                                                                                                                                                                                                                                                                                                                                                               |
| Malachite Green                                                                                                                                                                                                                                                                                                                                                                                                      | 657             |                                                                                                                                                                                                                                                                                                                                                               |
| 10 Rhodamine 6G                                                                                                                                                                                                                                                                                                                                                                                                      | 752             | 10                                                                                                                                                                                                                                                                                                                                                            |
| Rhodamine B                                                                                                                                                                                                                                                                                                                                                                                                          | 749             |                                                                                                                                                                                                                                                                                                                                                               |
| Methylene Violet                                                                                                                                                                                                                                                                                                                                                                                                     | 842             |                                                                                                                                                                                                                                                                                                                                                               |
| Direct colors reserved by the complex nitrogenous compounds                                                                                                                                                                                                                                                                                                                                                          |                 | 15                                                                                                                                                                                                                                                                                                                                                            |
| 15 Diphenyl Fast Yellow                                                                                                                                                                                                                                                                                                                                                                                              | 632             |                                                                                                                                                                                                                                                                                                                                                               |
| Benzo Fast Scarlet 8BS                                                                                                                                                                                                                                                                                                                                                                                               | 326             |                                                                                                                                                                                                                                                                                                                                                               |
| Paramine Orange                                                                                                                                                                                                                                                                                                                                                                                                      | 415             |                                                                                                                                                                                                                                                                                                                                                               |
| 20 Benzo Fast Orange WS                                                                                                                                                                                                                                                                                                                                                                                              | 326             | 20                                                                                                                                                                                                                                                                                                                                                            |
| Direct Blue 2B                                                                                                                                                                                                                                                                                                                                                                                                       | 406             |                                                                                                                                                                                                                                                                                                                                                               |
| Direct Sky Blue                                                                                                                                                                                                                                                                                                                                                                                                      | 520             |                                                                                                                                                                                                                                                                                                                                                               |
| Direct Blue RWS                                                                                                                                                                                                                                                                                                                                                                                                      | 512             |                                                                                                                                                                                                                                                                                                                                                               |
| Direct Pink                                                                                                                                                                                                                                                                                                                                                                                                          | 126             |                                                                                                                                                                                                                                                                                                                                                               |
| 25 Direct Black BH                                                                                                                                                                                                                                                                                                                                                                                                   | 401             |                                                                                                                                                                                                                                                                                                                                                               |
| The term "nitrogenous resin" as employed hereinafter in the claims is to be construed as including within its scope condensation products of gelatine, casein or other albumenoid compounds with formaldehyde or other aldehydes.                                                                                                                                                                                    |                 | 30                                                                                                                                                                                                                                                                                                                                                            |
| What I claim and desire to secure by Letters Patent is:—                                                                                                                                                                                                                                                                                                                                                             |                 |                                                                                                                                                                                                                                                                                                                                                               |
| 1. Process of coloring textile materials, which comprises impregnating at least part of the material with reagents capable of reacting to yield a nitrogenous resin and then effecting formation of compound from said reagents on the material, and dyeing the materials by applying a dyestuff to at least a portion of the impregnated 35 part at the earliest at the time of applying one of said reagents.      |                 |                                                                                                                                                                                                                                                                                                                                                               |
| 2. Process of coloring cellulosic textile materials, which comprises impregnating at least part of the material with reagents capable of reacting to yield a nitrogenous resin and effecting formation of said resin from said reagents on the material, and dyeing the materials by applying a dyestuff to at least a portion of the impregnated part at the earliest at the time of applying one of said reagents. |                 | 35                                                                                                                                                                                                                                                                                                                                                            |
| 3. Process of coloring textile fabric containing cellulose filaments, which comprises locally impregnating the fabric with reagents capable of reacting to yield a nitrogenous resin, effecting formation of said nitrogenous resin on the materials, and thereafter dyeing the material with a dyestuff having affinity for animal fibers.                                                                          |                 | 40                                                                                                                                                                                                                                                                                                                                                            |
| 4. Process of coloring textile fabric containing cellulose filaments, which comprises locally impregnating the fabric with a mixture of formaldehyde and a nitrogenous compound capable of                                                                                                                                                                                                                           |                 | 45                                                                                                                                                                                                                                                                                                                                                            |
|                                                                                                                                                                                                                                                                                                                                                                                                                      |                 | 50                                                                                                                                                                                                                                                                                                                                                            |
|                                                                                                                                                                                                                                                                                                                                                                                                                      |                 | 55                                                                                                                                                                                                                                                                                                                                                            |
|                                                                                                                                                                                                                                                                                                                                                                                                                      |                 | 60                                                                                                                                                                                                                                                                                                                                                            |

GEORGES RIVAT.

CERTIFICATE OF CORRECTION.

Patent No. 2,123,152.

July 5, 1938.

GEORGES RIVAT.

It is hereby certified that error appears in the printed specification of the above numbered patent requiring correction as follows: Page 3, first column, line 37, claim 1, before "compound" insert the word said; and that the said Letters Patent should be read with this correction therein that the same may conform to the record of the case in the Patent Office.

Signed and sealed this 9th day of August, A. D. 1938.

(Seal)

Leslie Frazer  
Acting Commissioner of Patents.